

Patented Feb. 17, 1925.

1,527,088

# UNITED STATES PATENT OFFICE.

EZEKIEL J. SHACKELFORD AND WILLIAM B. D. PENNIMAN, OF BALTIMORE, MARYLAND, ASSIGNORS TO RADIAC METALS, LTD., OF MASTERTON, NEW ZEALAND, A CORPORATION OF NEW ZEALAND.

## METHOD OF MAKING IRON-CHROMIUM ALLOYS.

No Drawing.

Application filed December 11, 1924. Serial No. 755,302.

To all whom it may concern:

Be it known that we, EZEKIEL J. SHACKELFORD and WILLIAM B. D. PENNIMAN, citizens of the United States, residing at Baltimore, State of Maryland, have invented an Improvement in Methods of Making Iron-Chromium Alloys, of which the following description is a specification.

This invention relates to the production 10 of low carbon alloys of iron and chromium, either by direct reduction of the chromium out of its ores or compounds into a bath of molten iron or steel, or by removal of the carbon from high carbon chromium iron 15 alloys (ferro chromes) made by the direct reduction process hereinafter described, or by other known processes. It relates in particular to (a) the production of stainless irons with chromium contents ranging from 20 8 to 20% and carbon contents from .05 to .15%; (b) stainless steels with chromium contents of 12 to 16% and carbon contents of .15 to 1.0%; and (c) ferro chromes with 45 to 65% chromium and .10 to 1.0% carbon. 25 Hitherto it has been common practice to make low carbon ferro chrome by first smelting chrome ore with carbon in an electric arc furnace or in a blast furnace to obtain a product with 40 to 65% chromium and 6 30 to 9% carbon. This high carbon material was then remelted in an electric furnace under a slag containing lime and iron ore, or chrome ore, in order to burn out the carbon. On account of the large amount of 35 carbon relative to the chromium, such methods cause high chromium losses, since chromium is removed from the metal being refined much faster than is carbon. A further disadvantage is that by such methods it is difficult and expensive to secure 40 ferro chromes with less than one or two per cent carbon. Thus, such methods are costly and give low grade products.

Other methods practiced commercially depend upon substituting the reducing action 45 of carbon by silicon, aluminum, calcium, or silicon carbides, and alloys of silicon and aluminum or of calcium and silicon. These methods give fairly low carbon ferro 50 chromes, but the cost is high, and objectionable amounts of silicon or aluminum are often left in the alloy.

In practicing the invention there may be utilized the various commercial forms of

carbon as reducing materials, in such ways 55 that there is a minimum contamination of the reduced metal by carbon. Consequently in the subsequent refining stages there is a relatively small amount of carbon to be removed and the chromiuim losses during 60 refining are correspondingly reduced. Furthermore, by working with a very active refining slag of small volume, the time of refining may be shortened, thus minimizing 65 still further the chromium losses.

In order to accomplish these results in the direct production of chromium from its ores the following features are advantageous, as will be more fully explained hereafter: (1) a rapid furnace capable of close temperature control; (2) sizing of reducing agents; (3) intimate mixture of ore and reducing material; (4) careful regulation of rate of feeding of the mixture to be smelted relative to the energy supplied the furnace; (5) 70 periodic removal of slag resulting from the reduction of the ore before accumulation of too great a slag volume; (6) complete removal of the smelting slag before adding the constituents of the refining slag; (7) a high 75 temperature and a small slag volume during the refining operation; (8) use of less carbon or other reducing agent than that needed for complete reduction of the chromium and iron oxides. 80

These steps in this process are based upon the following phenomena which have been observed during experiments. When chromium is reduced by carbon from its commercially available ores into a molten iron or 85 steel bath, slag is formed from the impurities in the ore and carbon; the volume of this slag increases with the amount of ore, and reducing agent fed in. The chromium content of the charge decreases and the 90 chromium content of the metal increases so long as the reducing agent is present in the ore mixture being fed in. It has been found, however, that as soon as the reducing agent disappears from the ore mixture, 95 the slag immediately begins to take out chromium and iron from the metal bath underlying it. If the temperature is high and the slag volume large, several per cent of chromium may disappear from the bath in 100 an hour. It has also been found that the carbon absorbed by the metal bath is minimized by (a) rapid reduction and smelting 105

of chrome ore in the ore—carbon mixture, so as to cut down the time the bath is exposed to carbon contamination; and (b) using somewhat less than the theoretical amount 5 of carbon needed to completely reduce the chromium ore charge.

In the decarbonizing phase it is found that a strongly basic decarbonizing slag as high as possible in chromium oxide is the 10 preferred condition, because such a slag, being already nearly saturated with chromium oxide, tends to rob the bath of but little chromium. We find that the activity of this 15 slag can be so increased by adjusting the temperature that its volume can be materially reduced over that hitherto customary, thus effecting further savings of chromium in the metal being refined.

Having now set forth briefly the procedure 20 and the experimental evidence on which it is based, there will now be described the direct reduction process by steps, as applied to the production of stainless steel or iron.

1. *Furnace*.—An arc furnace is preferred 25 of the arc-to-molten-bath type, with or without bottom electrode. The usual commercial forms of such furnaces may be used, but the preferred form should embody the following: 1. Two or more electrodes symmetrically disposed over the hearth; 2. Especially good electrode control so as to facilitate temperature adjustment; 3. Lines of furnace and its hearth volume so adjusted relative to the position and size of electrodes 30 35 that the furnace may be forced in order to facilitate the rapid working which characterizes this process; 4. Refractory lining and bottom chosen to withstand the corrosive action of the slags and the rapid working; 5. Customary facilities for introducing hot metal and for removing slags.

2. *The metal bath*.—For the production of stainless iron it is preferred to use molten blown metal from a Bessemer converter introduced into the electric furnace. Such metal should not carry more than .05% carbon.

For stainless steel the molten metal may be transferred from the converter to the 50 electric furnace before all its carbon is removed, say at 0.2% to 0.6% carbon.

If molten refined metal is not available from a Bessemer converter or an open-hearth furnace the bath can be formed by 55 melting and refining steel scrap in the electric furnace by means well known to the art. In any case, before charging the furnace with metal a limestone charge is first placed on the hearth of the furnace.

3. *Reception slag*.—As soon as the molten bath is formed it is covered with a reception slag composed of lime and fluorspar.

4. *Preparation of the mixed ore, flux and carbonaceous reducing material*.—As above stated, there is used finely crushed ore and

reducing material; this applies also to the flux. These ingredients are intimately mixed.

As a source of chromium there is employed commercial chromite or other chromium-rich materials. We have found 8 to 40 mesh a convenient size for the ore.

For reducing material ground, sized petroleum coke, ordinary coke or anthracite is preferred, although other carbon-rich materials may be used. All "fines" (i. e., materials passing a 60 mesh sieve) should be carefully eliminated, since it is found that retention of such fine reducing material causes upheavals and explosions in the rapid reduction process. The preferred size of the carbon particles is 8 to 20 mesh. The use of such sized reducing material has been found of great importance in promoting the rapid reduction of ore which is essential to success.

For fluxes silica, clay, rutile, ilmenite, fluorspar or lime, singly or in combination are used, according to the nature of the impurities in the ore and carbon reducing materials used. The aim is to secure a slag fluid enough, at the reduction temperatures used, to facilitate ready separation of reduced buttons of metal and the quick removal of the slag itself after disappearance of the reducing agent from the ore mixture.

5. *Charging the ore mixture*.—As soon as the reception slag is thoroughly fluid, the ore-flux-carbon mixture is introduced by shoveling, or by an ore charging machine. The mixture is spread thinly over the metal bath at such rate that there are never more than a few inches depth of unreduced mixture. A particular object of this method of charging is to minimize contact of carbon particles with the metal bath. The rate of charging is adjusted so as to carefully maintain this condition.

6. *Regulation of energy input of furnace*.—The electric energy passed into the furnace 110 is adjusted so as to give the maximum rate of reduction without, however, superheating to such an extent as to damage the roof or walls of the furnace. This energy input is naturally different for different furnaces, 115 and has to be ascertained for each furnace by trial. The object to be attained is to feed in ore mixture just as rapidly as it can be reduced and the reduced metal particles incorporated into the metal bath.

7. *Slagging off*.—Generally, it is advantageous to work as follows: After about one-half the ore mixture has been fed in, the energy input is slightly increased and the furnace operated until (a) the carbonaceous 125 particles have disappeared; (b) the slag has become fluid; and (c) the chromium content of the metal bath, as shown by quick chemical test or by fracture of a test piece, has reached a maximum. Immediately these 130

conditions are attained, the slag should be removed as rapidly and completely as possible.

8. *Continuation of ore charging.*—The 5 second portion of the charge is added in the same fashion as already described for the first; the testing of the bath and the slagging off being carried out as before. At the conclusion of this stage of the process the 10 metal will contain 10 to 20% chromium and rarely over 0.6% to 1.0% carbon. The time required for this step is usually three to four hours.

9. *Decarbonizing.*—Finely ground lime 15 and fluorspar are added to the bath immediately after removal of the last smelting slag, and the temperature is raised to a point where these additions melt in ten or fifteen minutes. Finely divided chromium 20 ore is then added gradually by shoveling, or by an ore charging machine, distributing it well over the surface of the bath. The high heat is continued with rapid chemical tests for carbon and chromium every ten minutes, 25 until the carbon content has been sufficiently reduced. Usually  $\frac{1}{2}$  to  $\frac{3}{4}$  hour is sufficient to reduce the carbon below 0.1%.

10. *Deoxidation.*—In order to remove oxides and gases from the bath, powdered ferro-silicon or ferro silicon aluminum, or other deoxidizing alloy, is strewn on the surface of the deoxidation slag. The amount to be added naturally varies with different heats and is adjusted by quick analysis of the metal bath for silicon or aluminum, or both, and by the appearance of fractured ladle tests. The aim is to prevent introduction of silicon or aluminum into the metal bath and to secure sound metal free from blow holes.

11. *Slagging off and tapping.*—Immediately after the chemical and fracture tests have shown that the above results have been attained, the decarbonization slag is removed as promptly as possible and the bath covered with powdered lime. The metal is allowed to stand in the furnace until at a proper temperature for tapping, after which it is transferred to a bottom-pour ladle and cast into ingots.

As a specific example of the application of the process the following is a description of the manufacture of stainless iron, without any limitation to the particular proportions or raw materials cited:

55 The operation may be conducted in any type of electric furnace which will permit the raising of the temperature of the contents to the desired degree. We used an 60 electric furnace of about three-quarter ton capacity, supplied with single phase alternating current, and having two depending electrodes arcing to the slag, the furnace lined with chrome brick free from carbon over the bottom and sides up to and above

the slag line; above the slag line, and for the roof was used a high grade refractory brick that was capable of withstanding the temperature. The area of the furnace at the slag line was approximately nine square 70 feet. In operating, molten iron or steel was poured in the furnace, and a basic slag melted thereon.

To a molten bath of 700 lbs. or iron carrying about 0.02% carbon there were added 75 35 lbs. lime and 15 lbs. fluorspar. The furnace at this stage was operated at 120 volts and 1200 amperes. After 15 minutes the lime and fluorspar were melted, forming the reception slag. The voltage was 80 maintained at 120 and the amperes at 1500, and approximately one-half the ore-carbon-flux mixture charged in by shoveling as already described. There were used 550 lbs. chromite ore, 117 lbs. coke carrying 12% 85 ash, and 12 lbs. fluorspar. After  $1\frac{1}{4}$  hours, all the ore was in, and after another  $1\frac{1}{4}$  hours, the first metal sample was taken for test. The electric energy supplied to the furnace was at the approximate rate of 90 from 600 to 700 watts per pound of chrome ore charged, and at the approximate rate of from 18000 to 22000 watts per square foot of slag surface. The slag was then 95 fluid and showed absence of coke granules; the metal bath showed 8.12% chromium. The slag was removed and the charging of the second portion of the ore-flux-carbon mixture begun, using the same current and voltage as on the first half. At the end of 100  $2\frac{1}{2}$  hours the slag appearance and the chromium content of the bath indicated that the slag should be removed. The decarbonizing slag was then formed by adding 15 lbs. lime and 10 lbs. fluorspar and melting by 105 the application of 120 volts and 2000 amperes for 15 minutes. Continuing with the same current conditions there were then added gradually 50 lbs. of chromium ore. The electric energy supplied during the decarbonizing stage was at the approximate rate 110 of 23000 to 28000 watts per square foot of slag surface. After 30 minutes, metal samples were taken every ten minutes for quick carbon determination. At the end of  $1\frac{3}{4}$  hours the carbon was 0.10% and the chromium 115 12.53%. Ten lbs. of powdered 50% ferrosilicon were then added and the slag removed after ten minutes. The current was shut off and powdered lime added as 120 described; the metal was then tapped into a ladle and cast into ingot molds. A ladle test of the finished metal showed .073% carbon, 12.52% chromium, and .12% silicon.

In the application of this process to the manufacture of low carbon ferrochrome the steps are substantially as described above, with, of course, suitable increases in the chromium ore, coke and flux additions, and decreases in the relative amount of low car-

bon in the initial bath. In decarbonizing, the ratio of slag volume to chromium content of the bath is kept substantially the same as in making stainless iron or stain-  
5 less steel.

In decarbonizing ferrochrome made by heretofore known processes, the same de-  
carbonizing principles are followed. It is,  
10 however, much preferable to use ferro-  
chrome made by the process described here-  
in since, as stated, it is initially much lower  
in carbon than that produced by the usual  
carbon reduction methods, and hence can be  
15 refined more economically to a low carbon  
product.

Having described the process and invention,  
what is claimed and desired to patent  
is:

1. The method of making iron-chromium  
20 alloys which comprises successively reduc-  
ing quantities of chrome ore in contact  
with a slag over a molten body of iron or  
steel, removing the slag periodically and  
supplying new slag material, of the same  
25 reducing character, and oxidizing the car-  
bon from the resulting chromium alloy by  
supplying a non-carbon charge after re-  
moving the reducing slag until the carbon  
is lowered to a permissible content.

30 2. The method of making iron-chromium  
alloys which comprises successively charg-  
ing and reducing quantities of chrome ore  
in contact with a slag over a molten body  
of iron or steel, removing the slag between  
35 the charges of chrome ore, oxidizing the  
carbon from the resulting chromium by a  
slag and chrome ore at a higher tempera-  
ture until the carbon is lowered to a per-  
missible content, and then deoxidizing the  
40 chromium alloy.

3. The method of making iron-chromium  
alloys which comprises melting a slag con-  
taining lime and fluorspar over a body of  
molten iron or steel, periodically charging  
45 a mixture of chrome ore, carbon, and fluo-  
spar upon said slag, reducing said chrome  
ore and periodically removing slag, oxidiz-  
ing the carbon from the resulting alloy by  
a slag and chrome ore at a higher tempera-  
50 ture until the carbon is lowered to a per-  
missible content, and deoxidizing the re-  
sulting alloy.

4. The method of making iron-chromium  
55 alloys which comprises melting a slag con-  
taining fluxing and refining agents, upon  
a body of molten iron or steel, periodically  
charging a mixture of chrome ore, carbon  
and fluorspar upon the surface of the slag,  
reducing said chrome ore, removing slag  
60 between the successive charges of chrome  
ore mixture, adding slag materials, raising  
the temperature of the mass with the suc-  
cessive additions of chrome ore mixture,  
oxidizing the carbon from the resulting  
65 chromium alloy by fresh slag material and

chrome ore at a higher temperature, and  
deoxidizing the resulting alloy.

5. The method of making iron-chromium  
alloys which comprises successively reduc-  
ing quantities of chrome ore associated with  
70 a reducing agent and slag material, over  
a molten body of iron or steel, supplying  
electric energy at the approximate rate of  
500 to 700 watts per pound of chrome ore  
charged, depending upon the size of the  
75 furnace and the charge therein, removing  
the slag periodically and supplying new  
slag material, oxidizing the carbon in the  
alloy formed at an increased temerature  
until the carbon is reduced to a permissible  
80 quantity, and withdrawing the alloy from  
the furnace.

6. The method of making iron-chromium  
85 alloys which comprises successively reduc-  
ing quantities of chrome ore associated with  
a reducing agent and slag material over a  
molten body of iron or steel, supplying elec-  
tric energy at the approximate rate of 500  
90 to 700 watts per pound of chrome ore  
charged, removing the slag periodically and  
charging additional quantities of chrome  
ore mixture periodically, maintaining the  
temperature in the furnace, withdrawing  
95 the slag and charging new slag material, in-  
creasing the temperature and charging  
chrome ore thereto, and maintaining the in-  
creased temperature until the carbon is re-  
duced to a permissible content, and with-  
drawing the alloy.

7. The method of making iron-chromium  
100 alloys which comprises successively reduc-  
ing quantities of chrome ore associated with  
a reducing agent and slag material over a  
molten body of iron or steel, supplying  
electric energy at the approximate rate of  
105 500 to 700 watts per pound of chrome ore  
charged, removing the slag periodically and  
charging additional quantities of chrome  
ore mixture periodically, maintaining the  
supply of electric energy to the furnace  
110 during the reduction period, withdrawing  
the slag after sufficient chrome ore has been  
reduced and charging new slag material,  
oxidizing the carbon in the alloy by the  
addition of chrome ore and a very con-  
115 siderable increase in the supply of electric  
energy to the furnace, thereby raising the  
temperature, and continuing the high tem-  
perature treatment until the carbon has  
been reduced to a permissible content.

8. The method of reducing chrome ore to  
chromium or chrome alloy, and making  
iron-chromium alloys, which comprises sup-  
plying a body of molten iron or steel with  
125 slag material, charging thereupon a quantity  
of chrome ore associated with a reducing  
agent and a flux, supplying electric energy  
at the approximate rate of 500 to 700 watts  
per pound of chromium charged, removing  
130 the slag periodically and charging addi-

- tional quantities of chrome ore mixture and slag material periodically, the electric energy supply being maintained at approximately 18000 to 22000 watts per square foot 5 of slag surface covered by chrome ore mixture, removing the slag after the reduction of the chrome ore, supplying new slag material, and oxidizing the carbon in the resulting alloy by additions of chrome ore and 10 increasing the supply of electric energy to the furnace, until the carbon is reduced to a permissible content.
9. The method of reducing chrome ore and of making iron-chromium alloys, which 15 comprises supplying a body of molten iron or steel with a quantity of chrome ore associated with a reducing agent and a flux, supplying electric energy as heat at the approximate rate of 18000 to 22000 watts per 20 square foot of slag surface until the chrome ore is reduced and a sufficient quantity of chromium has been alloyed with the iron or steel, periodically changing the slag and renewing the supply of chrome ore mixture, 25 and oxidizing the carbon from the resulting alloy by reacting thereon with an oxidizing slag and chrome ore with an increased supply of electric energy until the carbon is reduced to a permissible content.
- 30 10. The method of making iron-chromium alloys, which comprises supplying to a body of molten iron-containing metal a slag material, charging thereupon a quantity of chrome ore associated with a reducing agent, 35 supplying electric energy at the approximate rate of 18000 to 22000 watts per square foot of slag surface, periodically replenishing the supply of chrome ore and reducing agent and slag materials, oxidizing the carbon in 40 the resulting alloy by reacting thereupon with an oxidizing slag and chrome ore with an electric energy supply of approximately 25000 watts per square foot of slag surface, until the carbon is reduced to a permissible 45 content.
11. The method of making iron-chromium alloys, which comprises supplying to a body of molten iron-containing metal a slag material, charging thereupon a quantity of 50 chrome ore associated with a reducing agent, supplying electric energy at the approximate rate of 18000 to 22000 watts per square foot of slag surface, periodically replenishing the supply of chrome ore and reducing agent 55 and slag materials, oxidizing the carbon in the resulting alloy by reacting thereupon with an oxidizing slag and chrome ore with an electric energy supply of approximately 23000 to 28000 watts per square foot of slag 60 surface, until the carbon is reduced to a permissible content.
12. In the method of making iron-chromium alloys, the step of decarbonizing the same which comprises covering said alloy 65 with an oxidizing slag and supplying chrome ore thereto, and heating the same by supplying electric energy as heat at the approximate rate of 23000 to 28000 watts per square foot of slag surface until the carbon is reduced to a permissible content. 70
13. In the method of making iron-chromium alloys, the step of decarbonizing the same which comprises covering said alloy with a slag rich in chromium oxid and poor in iron oxid, supplying chrome ore thereto, 75 and heating the same by supplying electric energy as heat at the approximate rate of 23000 to 28000 watts per square foot of slag surface until the carbon is reduced to a permissible content. 80
14. The method of reducing chrome ore and of making iron-chromium alloys, which comprises supplying a body of molten iron or steel with a quantity of chrome ore associated with a reducing agent and a flux, 85 supplying electric energy as heat at the approximate rate of 18000 to 22000 watts per square foot of slag surface until the chrome ore is reduced and a sufficient quantity of chromium has been alloyed with the iron or steel, periodically changing the slag and renewing the supply of chrome ore mixture, and oxidizing the carbon from the resulting alloy by reacting thereon with an oxidizing slag and chrome ore with an increased supply of electric energy until the carbon is reduced to a permissible content and then deoxidizing the alloy. 90
15. The method of making iron-chromium alloys, which comprises supplying to a body of molten iron-containing metal a slag material, charging thereupon a quantity of chrome ore associated with a reducing agent, 95 supplying electric energy at the approximate rate of 18000 to 22000 watts per square foot of slag surface, periodically replenishing the supply of chrome ore and reducing agent and slag materials, oxidizing the carbon in the resulting alloy by reacting thereupon with an oxidizing slag and chrome ore with an electric energy supply of approximately 100 25000 watts per square foot of slag surface, until the carbon is reduced to a permissible content and then deoxidizing the alloy. 105
16. The method of making iron-chromium alloys, which comprises supplying to a body of molten iron-containing metal a slag material, charging thereupon a quantity of chrome ore associated with a reducing agent, 110 supplying electric energy at the approximate rate of 18000 to 22000 watts per square foot of slag surface, periodically replenishing the supply of chrome ore and reducing agent and slag materials, oxidizing the carbon in the resulting alloy by reacting thereupon with an oxidizing slag and chrome ore with an electric energy supply of approximately 115 23000 to 28000 watts per square foot of slag surface, until the carbon is reduced to a permissible content and then deoxidizing the alloy. 120
17. The method of making iron-chromium alloys, which comprises covering said alloy with an oxidizing slag and supplying 125 electric energy as heat at the approximate rate of 23000 to 28000 watts per square foot of slag surface until the carbon is reduced to a permissible content and then deoxidizing the alloy. 130

17. In the method of making iron-chromium alloys, the step of decarbonizing the same which comprises covering said alloy with an oxidizing slag and supplying 5 chrome ore thereto, and heating the same by supplying electric energy as heat at the approximate rate of 23000 to 28000 watts per square foot of slag surface until the carbon is reduced to a permissible content and then 10 deoxidizing the alloy.

18. In the method of making iron-chromium alloys, the step of decarbonizing the same which comprises covering said alloy

with a slag rich in chromium oxid and poor in iron oxid, supplying chrome ore thereto, 15 and heating the same by supplying electric energy as heat at the approximate rate of 23000 to 28000 watts per square foot of slag surface until the carbon is reduced to a permissible content and then deoxidizing the 20 alloy.

In testimony whereof, we have signed our names to this specification.

EZEKIEL J. SHACKELFORD.  
WILLIAM B. D. PENNIMAN.